

## UNITED STATES PATENT OFFICE.

AUGUST E. NIENSTADT, OF NEWARK, NEW JERSEY, ASSIGNOR OF ONE-HALF TO GEORGE H. ROSENBLATT, C<sup>o</sup> NEW YORK, N. Y.

## EXPLOSIVE.

No. 841,172.

Specification of Letters Patent.

Patented Jan. 15, 1907.

Application filed January 30, 1906. Serial No. 298,645.

*To all whom it may concern:*

Be it known that I, AUGUST E. NIENSTADT, a citizen of the United States of America, and a resident of Newark, county of Essex, and State of New Jersey, have invented certain new and useful Improvements in Explosives, of which the following is a specification.

This invention has reference to a novel explosive composition to be used in the arts and trades as a blasting-powder and a charge for cartridges for blasting or firearms.

Another application of the explosive composition is its use as a flashlight on water during the night in order to determine the exact location of distant objects—for instance, vessels, and particularly war vessels.

The explosive composition exists in form of powder. It consists of two active agents which when well mixed are inactive under normal conditions. When water or any aqueous solution is applied to the two active agents, they are decomposed in contact with the water, and an explosion results in closed places, or when the powder is thrown on water in shells or firearms or otherwise flames issue from the mixture and illuminate the neighborhood. In this way the location of a man-of-war may be determined at night. The two active agents are metallic sodium or potassium and calcium carbide. The metallic sodium decomposes water and liberates hydrogen. Likewise the calcium carbide is decomposed by water and produces per molecule one molecule of acetylene gas, which under certain conditions resolves itself into its component elements, carbon and hydrogen. Acetylene is an endothermic combination of two elements, and the heat absorbed in its production or its equivalent in other form of energy exists therein in latent form and reasserts itself upon provocation. In addition thereto some air is always present and when the hydrogen is ignited during the explosion the atomic carbon resulting from the decomposition of the acetylene gas is partly or wholly transformed into carbon mono or di oxid. These gases also increase the volume of the explosive gaseous mixture during the explosion.

If it is desired to have a less violent explosion, any other metal may be used in the

compound, provided same is capable of decomposing water under ordinary conditions—for instance, calcium.

The alkali metals, particularly sodium and potassium, possess the property of decomposing water under ordinary conditions to the highest known degree. Their affinity to oxygen is so great that these two metals oxidize immediately in the open air. The metals are soft and may be cut with an ordinary knife. When a small disk of the metal is cut off, the new surface of the disk remains shiny for a moment only. It is oxidized immediately. Therefore these metals are kept constantly under Pennsylvania oils in glass bottles during transportation and storage. These metals are so soft that they cannot be powdered in any manner or form like other metals.

I have discovered that the alkali metals may be safely reduced to powder in combination with calcium carbide. The latter is first preferably reduced to a coarse powder. Then the quantity of metal is mixed with the carbide so that the metal is covered by same. Now the mixture may be powdered in a mortar or in any other suitable machinery generally used in chemical works for reducing substances. The percentage of alkali metal in its native state in the composition varies from two per cent. to twenty-five per cent., while calcium carbide is used from seventy-five to about ninety-eight per cent. It is of course understood that any other percentage may be selected for specific uses. Metallic sodium may also be cautiously heated to the fusion-point. Then the calcium carbide is introduced and both stirred together. When cool, this mixture is then ground. In this instance the metal is found in the composition in a more finely divided state. The powder thus obtained may be stored in any kind of receptacle which is adapted to keep out moisture. It may be kept in glass bottles with ordinary rubber stoppers paraffined at the top, notwithstanding the fact that the otherwise dangerous metallic sodium is contained therein.

The resulting expandable explosive gases produced during the explosion consist of two kinds of explosive mixtures. The hydrogen, oxygen, and air is one, and the acety-

lene, air, and hydrogen the second. Furthermore, acetylene gas in a confined space before the explosion occurs will at a certain moment be compressed, and in a condensed state this gas is very unstable, and therefore more easily exploded, owing to the well-known relatively low critical temperature of same, which prevents its commercial liquefaction.

In the described manner I have provided a novel explosive which contains the normally dangerous alkali metals, particularly sodium, in their metallic state.

The explosive composition made of calcium carbide and the alkali metals in their metallic state may be safely transported and stored and when it comes in contact with water explodes and ignites spontaneously.

Having thus described my invention, I claim as new and desire to secure by Letters Patent—

1. The process of producing an explosive composition consisting in reducing calcium carbide to small particles, admixing it with a metal which is capable of decomposing water under ordinary conditions enveloping there-

by the metal by the coarse powder of calcium carbide, and reducing the mixture to powder.

2. The process of producing an explosive composition consisting in reducing calcium carbide to small particles, admixing therewith metallic sodium enveloping thereby the metallic sodium by the coarse powder of calcium carbide, and reducing the mixture to powder.

3. As a new article of manufacture a novel composition of matter composed of calcium carbide, and a metal in its uncombined state which is capable of decomposing water under ordinary conditions and existing in form of powder.

4. As a new article of manufacture a novel composition of matter composed of calcium carbide and metallic sodium and existing in form of powder.

Signed at New York, N. Y., this 27th day of January, 1906.

AUGUST E. NIENSTADT.

Witnesses:

LUDWIG K. BÖHM,  
GEORGE H. ROSENBLATT.